

May 10, 1932.

J. A. M. VAN LIEMPT

1,857,203

LEADING-IN CONDUCTOR

Filed March 13, 1930



Inventor:  
Johannes A.M. van Liempt,  
by *Charles V. Tullor*  
His Attorney.

## UNITED STATES PATENT OFFICE

JOHANNES ANTONIUS MARIA VAN LIEMPT, OF EINDHOVEN, NETHERLANDS, ASSIGNEE  
TO GENERAL ELECTRIC COMPANY, A CORPORATION OF NEW YORK

## LEADING-IN CONDUCTOR

Application filed March 13, 1930, Serial No. 435,586, and in the Netherlands November 30, 1929.

The present invention relates to the manufacture of incandescent lamps, electric discharge tubes of the transmitting type, gas-filled and vacuum rectifiers, X-ray tubes, etc., and more particularly to the leading-in conductors of such devices. 5

When conductors of the usual type are fused in an evacuated glass envelope, there may be air leakage in the region of each conductor. This leakage for the most part is believed to be due to the presence of small tears, fractures or fissures residing in the material of the conductor which structural failures cannot always be avoided in the prior art 15 sealing-in wires, notwithstanding the care taken during manufacture of the material. The tears may traverse the conductor material longitudinally or transversely and can usually be detected by metallographic methods. Leading-in conductor material is sometimes fabricated from a base metal such as tungsten, molybdenum or zirconium in powdered form and heated to a sintering temperature, simultaneously being pressed to shape 20 after which the body is hammered and drawn to wire size. Instead of a wire, the conductor may take the form of a tube which also may be drawn from the pressed and sintered body. Tungsten wire, which is frequently used for such material on account of its favorable coefficient of expansion when compared to that of Pyrex or other hard glass in which it may be sealed is particularly susceptible to failure of the crystal or 25 grain structure.

I have discovered and in accordance with my invention that when the various metals or alloys which heretofore have exhibited interstices or other forms of grain discontinuity or deformation are given a special treatment to form the multi-crystal structure into uni-crystalline, i. e. from a microcrystal to a macrocrystal state, the metal takes on the character of being strongly resistant to tear 40 and may be satisfactorily employed as leading-in conductor material for sealing into a boro-silicate glass. Metal treated in the manner described presently is found to have a dense, coherent section which positively precludes gas or air leakage, even after long 45

periods of time. The invention thus has application to all types of high vacuum devices, particularly to the power type which necessitates stems of hard glass, also to gas-filled rectifiers and ordinary incandescent lamps in which air leakage causes substantial reduction of operating life. 55

Various methods of changing the micro-crystalline metallic structure into macro-crystalline are well known in the art, and it will be sufficient to cite as one example the immersion of the sealing-in material in an atmosphere of tungsten chloride (WCl<sub>6</sub>). A process of this kind has been described by Van Arkel in the Dutch Journal Physika, 60 1923, Vol. II, at page 76.

The drawing illustratively exemplifies the application of the invention to a rectifier. In the figure, numeral 1 designates an envelope of boro-silicate glass which may be evacuated or filled with inert gas of suitable pressure, the envelope terminating in a stem 2. Within the envelope there is a filamentary electrode 3 and a cooperating anode 4. Leading-in conductors 5 are sealed in the stem for supplying current to the electrodes. These conductors may be fabricated of any refractory metals, such as tungsten, molybdenum or zirconium which has a favorable coefficient of expansion as compared to that of the glass 65 in which it is sealed and may be treated in any well known and appropriate manner to change the grain structure from the usual microcrystal formation to macrostrystalline. 70

What I claim as new and desire to secure by Letters Patent of the United States is:—

1. In combination, an evacuated envelope, a conductor within the envelope and a metallic member sealed in the envelope for supplying current to said conductor, said member having a uni-crystalline structure whereby gas leakage through the envelope in the region of the metallic member is prevented. 80

2. An evacuated envelope terminating in a stem, a conductor within the envelope and a metallic member sealed in said stem for supplying current to the conductor, said member having a uni-crystalline structure whereby gas leakage through the stem in the region of the metallic member is prevented. 85

100

3. An evacuated envelope terminating in a stem and constituted of boro-silicate glass, one or more conductors within the envelope and tungsten wires sealed in said stem for supplying current to the conductors, said tungsten wires being macrocrystalline.

In witness whereof, I have hereunto set my hand and seal this twentieth day of February, 1930.

10 JOHANNES ANTONIUS MARIA van LIEMPT.

- 18

20